

1

3,122,457

## PROTECTIVE COATING FOR MAGNESIUM AND ZINC

Herbert K. De Long and James A. Brown, both of Midland, Mich., assignors to The Dow Chemical Company, Midland, Mich., a corporation of Delaware  
No Drawing. Filed Sept. 18, 1961, Ser. No. 138,620  
6 Claims. (Cl. 148—6.21)

This invention relates to an improved coating for magnesium and zinc articles and to a method for producing such a coating. It more particularly is concerned with a surface conversion coating for magnesium and zinc which renders these metals resistant to corrosive attack.

The term "magnesium" as used herein refers to magnesium metal or a magnesium-base alloy which contains about 85 percent or more magnesium. The term "zinc" as used herein refers to zinc metal or a zinc-base alloy which contains about 85 percent or more zinc. The term "chromate-manganate coating" as used herein refers to a coating which is formed by subjecting magnesium and zinc articles to the action of a solution containing a chromium compound and a manganese compound in an acidic aqueous solution containing sulfate ions and which is thought to contain chromate ions ( $\text{CrO}_4^{2-}$ ) and manganate ions ( $\text{MnO}_4^-$ ) as constituents. Such a coating imparts corrosion-resistant properties to these articles.

Many conventional coating solutions and coatings formed on magnesium and zinc by immersion in, or brush-application of, aqueous solutions containing chromium compounds have been unsatisfactory in a number of particulars. Variations in the color of the coated article, lack of uniformity of thickness of the coating, formation of powdery material on the coating during the coating process, failure to build up a coating of desired thickness, and high metal loss are some of the disadvantages encountered in the use of known coating solutions. Furthermore, in many of the processes for forming chromate coatings the accumulation of altered chromium and magnesium or zinc compounds in the bath during usage necessitates discarding and replacing the bath at uneconomically frequent intervals.

It is a principal object of the present invention to provide an improved chromate based surface conversion coating which can be used on both magnesium and zinc. It is another object of the present invention to provide a method for producing a surface conversion coating of uniform color. A further object of the present invention is to provide a chromate coating solution which is economical of active ingredients and has a long service life. A still further object is to provide a solution for chromate coating which undergoes very little build up of undesirable compounds and which may be revived by mere addition of active ingredients to the solution and therefore need not be discarded after relatively short periods of use. It is an additional object of the present invention to provide a novel chromate-manganate undercoating for magnesium and zinc articles and particularly pressure die-cast articles which is an excellent base for paint coatings. These and other objects and advantages will become apparent from the detailed description presented hereinafter.

This invention is based upon the discovery that specific acidic aqueous chromate-manganate solutions in the presence of sulfate will produce a surface conversion coating on magnesium and zinc base articles which coating has a desirable uniformity of color and thickness and high resistance to corrosion.

The aqueous acidic chromate-manganate bath of the present invention comprises on a weight basis from about 2 to about 25 percent and preferably from about 12 to about 18 percent chromate expressed as  $\text{Na}_2\text{Cr}_2\text{O}_7 \cdot 2\text{H}_2\text{O}$ , from about 0.05 to about 1 and preferably from about 0.3

2

to about 0.6 percent manganate expressed as  $\text{KMnO}_4$ , from about 0.2 to about 0.55 percent and preferably about 0.36 to about 0.45 percent sulfate, expressed as 98 percent  $\text{H}_2\text{SO}_4$ , and will have a pH of from about 0.9 to about 1.8 and preferably between about 1 and 1.7.

The bath is operated at a temperature of from about 50 to about 140° F. and preferably from about 70 to about 110° F.

The chromate can be supplied by a water soluble dichromate, e.g. sodium dichromate, potassium dichromate and ammonium dichromate.

Sodium permanganate and potassium permanganate are the preferred forms for supplying the manganate.

Sulfuric acid (98 percent  $\text{H}_2\text{SO}_4$ ) is a very satisfactory means for supplying the small amount of sulfate ion utilized in the bath as well as helping to maintain the pH of the solution within the operable range. To illustrate, 1 and 3 milliliters of 98 percent  $\text{H}_2\text{SO}_4$  per liter of solution are equivalent to about 0.2 and about 0.55 weight percent  $\text{SO}_4^{2-}$  respectively in the treatment bath.

In practicing the invention, the article to be coated is degreased, if necessary, by a conventional degreasing method. The degreasing step conventionally consists of immersing the article in or rubbing it with an aqueous alkaline solution, e.g., a water solution of sodium carbonate and sodium hydroxide. The degreased magnesium is thereafter rinsed free of residual alkali with water and dried.

With magnesium articles, the degreasing step may be followed by an activation step or they may be immersed without further preparation in the novel coating solution of the present invention. Activation consists of activating the surface of the magnesium, i.e., making it a more receptive site upon which to form the chromate coating.

The activation may be carried out by one of several ways. One effective way is to prepare a 0.5 percent by volume aqueous solution of 30 weight percent aqueous hydrofluosilicic acid or a 0.5 percent by volume aqueous solution of 50 weight percent hydrofluoric acid and to immerse the magnesium article in this solution at about room temperature or a little above, i.e. about 70° to 90° F. Immersion in the hydrofluosilicic acid solution should be for about 0.5 minute and immersion in the hydrofluoric acid be from about 0.5 to about 2 minutes and preferably for about one minute.

If desired, for magnesium the degreasing and activating steps may be combined in a single step. Either of the two solutions, A and B set out below, will serve as a bath in which the magnesium may be immersed in a combined step. The bath temperature should be about 175° to about 185° F. and the duration of the immersion between about 1 and 5 minutes, but preferably about 2 minutes.

*Solution A.*—50 grams of tetrkasodium pyrophosphate ( $\text{Na}_4\text{P}_2\text{O}_7$ ) and 20 grams of sodium metaborate ( $\text{Na}_2\text{BO}_3 \cdot 2\text{H}_2\text{O}$ ) dissolved in sufficient water to make 1 liter of solution at room temperature.

*Solution B.*—70 grams of sodium tetraborate or borax ( $\text{Na}_2\text{B}_4\text{O}_7 \cdot 10\text{H}_2\text{O}$ ), 40 grams of tetrkasodium pyrophosphate ( $\text{Na}_4\text{P}_2\text{O}_7$ ) and 15 grams of sodium fluoride ( $\text{NaF}$ ) dissolved in sufficient water to make 1 liter of solution at room temperature.

The activating step is completed by rinsing the magnesium article well with water.

After the degreasing step, or the degreasing and activating steps if both are used with magnesium, the article is treated by immersing from about 10 to about 90 seconds and preferably from about 15 to about 30 seconds in the acidic aqueous chromate-manganate bath of the present invention.

After treatment in the chromate-manganate solution the article may be water-rinsed and dried.

The chromate-manganate solution of the invention may

be used over a long period of service by additions at intervals of the active ingredients therein.

The following examples will serve to illustrate further the present invention but are not meant to limit it thereto.

#### EXAMPLE 1

A 4 by 6 inch die-cast panel of AZ91B magnesium alloy as designated by ASTM nomenclature (nominal composition 9 percent aluminum, 0.15 manganese and 0.7 percent zinc) was degreased by immersing for about 3 minutes at 170° F. in a solution prepared by dissolving 40 grams of tetrasodium pyrophosphate, 70 grams borax and 15 grams sodium fluoride in sufficient water to make a liter of solution. The so-treated panel was removed from the solution, rinsed with hot water for about 15 seconds at 180° F. and then rinsed with cold water. The rinsed panel was thereafter immersed for 15 seconds at about 75° F. in the novel aqueous chromate-manganate solution of the invention having a pH value of 1.15, containing the following active constituents or ingredients:

Sodium dichromate ( $Na_2Cr_2O_7 \cdot 2H_2O$ ) (180 grams per liter)

Potassium permanganate ( $KMnO_4$ ) (5 grams per liter)

Sulfuric acid (98 percent  $H_2SO_4$ ) (2.5 mol. per liter)

The so-treated panel was removed from the solution, rinsed well with cold water, followed by a hot water rinse for 10 seconds at 150° F. and force dried for 10 minutes at 225° F.

A very good uniform light brown adherent and non-powdery coating was produced on the panel by this procedure. A number of die-cast panels were treated in the present solution and these were tested in high humidity and exterior corrosion type test medium using panels having bare untreated surfaces as controls. Other panels having the instant chromate-manganate conversion coating were painted using an automotive paint system and these panels were also treated in high humidity and salt spray corrosion tests. The results of these tests are shown in Table I.

Table I  
UNPAINTED

| Unpainted Condition Treatment | Percent Surface Corrosion or Oxidation      |                                        |
|-------------------------------|---------------------------------------------|----------------------------------------|
|                               | 100 Hrs. in 95% Relative Humidity at 95° F. | 3 Months' Industrial Exterior Exposure |
| Chromate-Manganate            | 1/2% Corrosion and No Oxidation.            | 3% Corrosion and No Oxidation.         |
| No treatment (control)        | 5% Corrosion and 85% Oxidation.             | 10% Corrosion and 100% Oxidation.      |

#### PAINTED<sup>1</sup>

| Treatment          | 20% Salt Spray at 95° F. (500 Hrs.) Corrosion, Percent |         | 95% Relative Humidity at 95° F. Paint Blistering—Paint Blistering, Percent—100 Hours |
|--------------------|--------------------------------------------------------|---------|--------------------------------------------------------------------------------------|
|                    | Scribe                                                 | General |                                                                                      |
| Chromate-Manganate | 1                                                      | 1/2     | 1                                                                                    |
| No treatment       | 100                                                    | 10      | 80                                                                                   |

<sup>1</sup> Paint system—1 coat of a modified alkyd yellow zinc chromate primer baked 25 mins. at 250° F. plus 1 coat of a modified alkyd dark gray low gloss metallic topcoat baked 25 mins. at 250° F.

#### EXAMPLE 2

Panels of AZ31B magnesium alloy (nominal composition 3 percent aluminum, .04 percent manganese and 1 percent zinc) were precleaned and given the chromate-manganate treatment following the procedures and using solution concentrations as described in Example 1 using a 30 second immersion time in the chromate-manganate bath. A uniform brown adherent coating was obtained

by this procedure. The so-treated AZ31B magnesium alloy extruded panels were compared in high humidity, salt spray and industrial exterior exposure corrosion type of testing with or without paint using as controls bare AZ31B panels which have not been given the chromate-manganate treatment. The results of these tests are shown in Table II.

Table II  
UNPAINTED

| Chemical Treatment | Percent Surface Corrosion or Oxidation     |                          |                                  |
|--------------------|--------------------------------------------|--------------------------|----------------------------------|
|                    | 95% Relative Humidity at 95° F. (100 Hrs.) | 20% Salt Spray (24 Hrs.) | Industrial Exterior Exp. (1 mo.) |
| Chromate-Manganate | OK                                         | 50% Corrosion.           | 2% Corrosion.                    |
| None (control)     | 100% Oxidation                             | 80% Corrosion.           | 90% Corrosion.                   |

#### PAINTED<sup>1</sup>

| Chemical Treatment | 95% Relative Humidity at 95° F., Percent Paint Blistering (1,000 Hrs.) | 20% Salt Spray, Percent Corr. (1,000 Hrs.) |      | Ind. Ext. Exp. Paint Adhes., 1 Month |
|--------------------|------------------------------------------------------------------------|--------------------------------------------|------|--------------------------------------|
|                    |                                                                        | Scribe                                     | Gen. |                                      |
| Chromate-Manganate | 6                                                                      | 15                                         | OK   | Good.                                |
| None               | 30                                                                     | 20                                         | OK   | Good.                                |

<sup>1</sup> Paint system—1 coat of a polyvinyl butyral zinc chromate primer baked 20 mins. at 300° F. plus 2 coats of Mil-E-7729 alkyd white gloss enamel force dried 2 hours at 160° F.

#### EXAMPLE 3

Example of the application of the chromate-manganate treatment to zinc base die castings.

Zinc alloy (ASTM AG40A alloy—Al—4%, Cu—0.25%, Mg—0.03%, balance Zn) die castings were treated by the following procedure.

(1) Alkaline cleaned 3 mins. in 6% trisodium phosphate at 200° F.

(2) Cold water rinsed.

(3) Immersed 15 secs. in the chromate-manganate treatment using the same solution as was used in the previous examples.

(4) Cold water rinsed.

(5) Hot water rinsed 15 secs. at 150° F.

(6) Force dried 10 mins. at 225° F.

The above chromate-manganate treated zinc die castings and chromate treated zinc die castings treated with a commercial chromate treatment used for zinc die castings were painted with one coat of a modified alkyd zinc chromate primer baked for 25 mins. at 250° F. plus one coat of an alkyd dark gray low gloss metallic topcoat baked 25 mins. at 250° F. or given a single coat of the alkyd topcoat. The castings were then exposed to accelerated corrosion tests in 95 percent relative humidity at 95° F. to check paint blistering due to corrosion and/or inferior paint adhesion. The results of this test are shown in Table III which follows:

Table III

| Chemical Treatment                         | Paint Topcoat       | Paint Blisters (100 hrs.) |
|--------------------------------------------|---------------------|---------------------------|
| Chromate-Manganate                         | Primer plus topcoat | None.                     |
| Do.                                        | Topcoat alone       | None.                     |
| Commercial Chromate Treatment <sup>1</sup> | Primer plus topcoat | 5                         |
| Do.                                        | Topcoat alone       | 6                         |

<sup>1</sup> Commercial chromate treatment for zinc die castings based on sodium dichromate and sulphuric acid.

In a manner similar to the foregoing examples, a chromate-manganate treatment bath can be prepared utilizing about 245 grams  $K_2Cr_2O_7$ , about 8.5 grams

NaMnO<sub>4</sub> and about 3 cubic centimeters of 98 percent H<sub>2</sub>SO<sub>4</sub> per liter of solution. Also the bath can be prepared utilizing about 24 grams (NH<sub>4</sub>)<sub>2</sub>Cr<sub>2</sub>O<sub>7</sub>, about 1 gram KMnO<sub>4</sub> and about 1 cubic centimeter of 98 percent H<sub>2</sub>SO<sub>4</sub> per liter of solution.

Various modifications can be made in the present invention without departing from the spirit or scope thereof for it is understood that we limit ourselves only as defined in the appended claims.

We claim:

1. A composition for forming a protective surface coating on magnesium articles and zinc articles consisting essentially of an aqueous solution containing as effective constituents based upon the weight of the solution between about 2.0 and 25.0 weight percent chromate ion expressed as Na<sub>2</sub>Cr<sub>2</sub>O<sub>7</sub>·2H<sub>2</sub>O, about .05 to about 1 weight percent of manganate ion expressed as KMnO<sub>4</sub> and about 1 to 3 milliliters of sulfuric acid per liter of solution, said sulfuric acid containing about 98 percent H<sub>2</sub>SO<sub>4</sub>.

2. A composition for forming a protective surface coating on magnesium articles and zinc articles consisting essentially of an aqueous solution containing as effective constituents based upon the weight of the solution between about 12 and 18 percent of chromate ion expressed as Na<sub>2</sub>Cr<sub>2</sub>O<sub>7</sub>·2H<sub>2</sub>O, about 0.3 to about 0.6 percent manganate ion expressed as KMnO<sub>4</sub>, and about 2 to 2.5 milliliters of 98 percent H<sub>2</sub>SO<sub>4</sub> containing sulfuric acid per liter of solution.

3. In a method of producing a coating on an article composed of at least 85 percent magnesium, the step which consists of subjecting, at a temperature of from about 50 to about 140° F., the article, for a period of between 10 and 90 seconds, to the action of an aqueous solution having a pH between 0.9 and 1.8, said solution containing as effective constituents based upon the weight of the solution between about 2 and 25 percent of chromate ion expressed as Na<sub>2</sub>Cr<sub>2</sub>O<sub>7</sub>·2H<sub>2</sub>O, between about .05 and 1 weight percent of manganate ion expressed as KMnO<sub>4</sub> and about 0.2 to about 0.55 percent sulfate ion expressed as 98 percent sulfuric acid.

4. In a method of producing a coating on an article composed of at least 85 percent zinc, the step which consists of subjecting, at a temperature of from about 50 to about 140° F. the article, for a period of between 10 and 90 seconds, to the action of an aqueous solution having a

pH between 0.9 and 1.8, said solution containing as effective constituents based upon the weight of the solution between about 2 and 25 percent of chromate ion expressed as Na<sub>2</sub>Cr<sub>2</sub>O<sub>7</sub>·2H<sub>2</sub>O, between about .05 and 1 weight percent of manganate ion expressed as KMnO<sub>4</sub> and about 0.2 to about 0.55 percent sulfate ion, expressed as 98 percent sulfuric acid.

5. In a method of producing a coating on an article composed of at least 85 percent magnesium, the step which consists of subjecting the article, for a period of time between about 15 and 30 seconds and at a temperature of from about 70 to 110° F. to the action of an aqueous solution of pH between about 1 to 1.7, said solution containing as effective constituents, based upon the weight of the solution, between about 12 and 18 percent of chromate ion expressed as Na<sub>2</sub>Cr<sub>2</sub>O<sub>7</sub>·2H<sub>2</sub>O, about 0.3 to about 0.6 percent manganate ion expressed as KMnO<sub>4</sub> and about 0.36 to about 0.45 percent sulfate ion expressed as 98 percent sulfuric acid.

6. In a method of producing a coating on an article composed of at least 85 percent zinc, the step which consists in subjecting the article, for a period of time between about 15 and 30 seconds and at a temperature of from about 70 to 110° F. to the action of an aqueous solution of pH between about 1 to 1.7, said solution containing as effective constituents, based upon the weight of the solution, between about 12 and 18 percent of chromate ion expressed as Na<sub>2</sub>Cr<sub>2</sub>O<sub>7</sub>·2H<sub>2</sub>O, about 0.3 to about 0.6 percent manganate ion expressed as KMnO<sub>4</sub> and about 0.36 to about .45 percent sulfate ion expressed as 98 percent sulfuric acid.

#### References Cited in the file of this patent

#### UNITED STATES PATENTS

|           |                |               |
|-----------|----------------|---------------|
| 2,352,076 | Bushrod -----  | June 20, 1944 |
| 2,465,443 | Gide -----     | Mar. 29, 1949 |
| 2,480,448 | Coates -----   | Aug. 30, 1949 |
| 2,681,873 | Deniston ----- | June 22, 1954 |

#### FOREIGN PATENTS

|         |                     |               |
|---------|---------------------|---------------|
| 510,353 | Great Britain ----- | July 24, 1939 |
|---------|---------------------|---------------|

#### OTHER REFERENCES

Metallurgia, February 1951, pp. 53-61; p. 58, FIG. 8, curve 4, relied on.

UNITED STATES PATENT OFFICE  
CERTIFICATE OF CORRECTION

Patent No. 3,122,457

February 25, 1964

Herbert K. De Long et al.

It is hereby certified that error appears in the above numbered patent requiring correction and that the said Letters Patent should read as corrected below.

Column 3, line 25, for "mol." read -- ml. --.

Signed and sealed this 27th day of October 1964.

(SEAL)  
Attest:

ERNEST W. SWIDER  
Attesting Officer

EDWARD J. BRENNER  
Commissioner of Patents